

## UNITED STATES PATENT OFFICE

2,515,186

## AGE HARDENABLE NICKEL ALLOYS

Clarence George Bieber and Mortimer Pierce  
 Buck, Huntington, W. Va., assignors to The International Nickel Company, Inc., New York, N. Y., a corporation of Delaware

No. Drawing. Original application January 13, 1941, Serial No. 374,208. Divided and this application June 7, 1941, Serial No. 397,080

2 Claims. (Cl. 75—170)

1

The present invention relates to nickel alloys, and, more particularly, to age hardenable nickel-copper alloys.

It is among the objects of our invention to produce nickel alloys capable of being hardened by heat treatment to any selected hardness over a broad hardness range; to provide nickel alloys having maximum hardness in the aged condition commensurate with satisfactory forgeability and good machining properties; and to produce nickel alloys having a broad range of hot malleability combined with high mechanical properties in the age hardened condition.

Other objects and advantages of the present invention will become apparent from the following description of the present invention.

Generally speaking, the present invention is based upon the surprising discovery made by us that nickel base alloys containing copper and having among other desirable properties an advantageous combination of hot malleability, good machining properties, good response to heat treatment and high hardness in the heat treated condition can be produced by incorporating aluminum with both titanium and silicon in the alloy in critical amounts depending upon the nickel content, as hereinafter described. Response to heat treatment can be obtained in copper-containing nickel base alloys by incorporating only one of the elements aluminum, titanium or silicon in the alloy but the amount of hardening element necessary to produce maximum response to heat treatment is relatively large and this is accompanied by working difficulties. We have made the surprising discovery that by using aluminum in combination with silicon and titanium, the response to heat treatment with a smaller total amount of hardening element is as satisfactory or even better than in alloys containing only one of these hardening elements in effective amounts, and the new alloys are characterized by greatly improved hot malleability as compared with alloys of otherwise substantially the same composition containing only one of the hardening elements.

The nickel content of the alloys embodying the present invention in all cases will be at least 45% by weight of the alloy and usually will be 50% or substantially more than 50%. Copper will be present in amounts up to 45% of the alloy.

The relative amounts of aluminum, silicon and titanium may vary over a range of several percent provided the ratio of nickel to the hardener content is maintained within the limits defined herein. Aluminum and at least one of the ele-

2

ments of the group titanium and silicon must each be present in the alloy in amounts greater than 0.25%. The third hardening element may be present in amounts more or less than 0.25%, the essential feature of this invention being that at least two of the hardening elements must be present in amounts greater than 0.25%. Aluminum and silicon may be used in amounts up to about 5% of either, while titanium should be employed in amounts less than 2%. Titanium exerts its greatest effect in combination with the aluminum when present within the range of about 0.25% to less than 1%.

We have discovered that within the preferred titanium range the optimum range of hot malleability, hardenability and high hardness in the heat treated condition is obtained when the ratio of nickel to the sum of the aluminum, 2.3 times the titanium and the silicon is approximately 15, preferably within the range of 13 to 17, and always within the range of 11 to 20. Since the ratio is a quotient, it is immaterial what unit of weight is used to express the content of nickel, aluminum, titanium and silicon. Thus, for example, the amounts of these ingredients in any given alloy may be expressed in parts by weight, percentage by weight, etc., without changing the ratio.

The mechanical properties of the nickel-copper alloys having combinations of the hardening elements contemplated by the present invention are, to a considerable extent, improved by the presence of carbon, provided the carbon is present in amounts less than about 0.5%. The beneficial effect of carbon in the alloys containing aluminum and titanium is surprising in view of the known detrimental effect of carbon on nickel alloys containing titanium as substantially the only hardening element.

The adverse effect of carbon on the hardenability of alloys containing titanium as substantially the only hardening element is believed to be due to the formation of an inert titanium carbide which decreases the hardening efficiency of the titanium or destroys its hardening ability. The fact that carbon has a beneficial effect on alloys of the present invention is believed to indicate that the inert titanium carbide does not form in a substantial amount when aluminum is present with titanium, provided carbon is less than about 0.5% and preferably does not exceed about 0.35%. For general applications it is preferred to have carbon present in amounts between about 0.15 to 0.2%, although higher amounts may be present. If carbon exceeds

about 0.2%, precipitation of graphitic carbon may occur. The presence of graphitic carbon greatly improves the machinability of the alloy and is desirable where free machining properties are required, although the presence of precipitated carbon tends to lower the ductility somewhat. For free machining nickel-copper alloys the carbon content preferably is about 0.2% to 0.3%.

In the commercial production of alloys embodying the present invention, the composition ordinarily will fall within the following ranges:

| Element  | Per cent  |
|----------|-----------|
| Aluminum | 0.25- 5   |
| Titanium | 0.25- 2   |
| Silicon  | 0.25- 2   |
| Carbon   | 0.03- 0.5 |
| Copper   | 10- 45    |
| Nickel   | Balance   |

Manganese and iron may be present in the alloy in amounts not exceeding about 2% and 10% respectively. In commercial alloys of the present invention these elements usually are present in small amounts. Ordinarily, manganese will not exceed about 0.5% and may be as low as 0.25%

metal from the group silicon and titanium manufactured in accordance with the present invention are less susceptible to loss of strength and/or ductility after exposure for long periods of time at temperatures of approximately 500° F. to approximately 1100° F. than comparable alloys hardened by one of the elements alone. The new alloys retain their high properties at elevated temperatures, for instance, at steam temperatures of about 1000° F.

The titanium-bearing material possesses improved hot ductility and strength without detrimental effect upon other mechanical properties or the method of heat treatment necessary to procure the mechanical properties. The alloys of the present invention possess improved hot ductility within the hot working range of about 1400° F. to about 2300° F. The differences in hot ductilities of the titanium-free and the titanium-bearing alloys contemplated by the present invention are very pronounced. For example, a titanium-bearing alloy had a hot malleable range of about 800° F. or more, whereas a titanium-free alloy had a hot malleable range of only about 400° F. Data from typical melts are given in Table I.

Table I

| Material         | Malleable Range, Degrees F. | T. S. | Y. P. | B. H. | R. A., Per Cent | El., Per Cent |
|------------------|-----------------------------|-------|-------|-------|-----------------|---------------|
| Titanium-free    | 1,900-2,300                 | 136   | 82    | 212   | 41              | 31            |
| Titanium-bearing | 1,500-2,300                 | 167   | 126   | 321   | 37              | 26            |

T. S. = tensile strength in thousand pounds per square inch.

Y. P. = yield point in thousand pounds per square inch.

or even 0.05%. Iron ordinarily will be less than about 1% and may be present in amounts as small as 0.2% or even 0.05%. Iron and manganese apparently affect the base alloy only and do not affect the response of the alloy to heat treatment.

The alloys of the present invention can be heat treated in accordance with the technique developed by Mudge and described in U. S. Patents Nos. 1,755,554 through 1,755,557, or in accordance with the process of our prior application, Serial No. 253,350, now Patent No. 2,234,955 dated March 18, 1941. Generally speaking, the articles are heat treated subsequent to mechanical working, machining and forming operations, but under certain conditions the articles may be heat treated before the final operations. For example, fine spring wires may be cold drawn after the hardening heat treatment since this procedure develops the highest mechanical properties attainable in the material. It also produces finished material with a higher luster than can be developed in material which is heat treated after cold drawing. Finished machining may also be carried out after the heat treatment to eliminate any discoloration and warping which may occur during heat treatment. Heat treated material may be subjected to subsequent machining, stamping, or other fabricating operations whenever necessary.

Hot rolled material having the composition contemplated by the present invention will heat treat to Brinell hardnesses in excess of about 265, and about 300 Brinell represents an average value. Cold drawn or cold worked material in small sections, e. g., up to about one inch in sectional thickness, generally heat treats to Brinell hardness values of about 325 or more.

Nickel-copper alloys containing aluminum and

40 It will be seen from the foregoing description and the specific examples that we have provided nickel alloys combining optimum response to heat treatment with hot malleability. These alloys may be used for various articles of manufacture including rollers and bearing balls, bearing and races therefor, roller chains, drop forgings and tie rods for airplane construction, valve seats and other valve parts, pump rods and the like, pump rod sleeves, pump pistons for high pressures and temperatures, plungers, turbine blades, turbine diaphragm blading, lock washers, screws and nuts, tools, cutting blades and the like, pins and needles, spring and other resilient elements, airplane instrument parts, nozzles for burners, rods, sheets, strip, wire, bars, rolled shapes, etc.

55 The present application is a division of our prior copending application Serial No. 374,208 filed January 13, 1941, and which itself is a continuation in part of our prior application, Serial No. 253,350, filed January 28, 1939, and which issued on March 18, 1941, as Patent No. 2,234,955.

60 The present invention is not to be confused with our said prior Patent No. 2,234,955. It is to be observed that the present invention involves the discovery that a critical ratio of the nickel content to the content of aluminum, titanium and silicon must be maintained within the critical limits disclosed and claimed herein in conjunction with the special composition set forth in the specification and claims.

65 Although the present invention has been described in conjunction with preferred embodiments, it is understood that modifications and variations may be resorted to without departing from the spirit and scope of the invention, as those skilled in the art will readily understand.

We claim:

70 1. A free machining, age hardenable alloy con-

taining 10% to 45% copper, over 0.25% and up to 5% aluminum, over 0.25% and less than 1% titanium, 0.25% to 2% silicon, 0.2% to 0.3% carbon, 0.05% to 2% manganese, 0.05% to 10% iron, and the balance substantially all nickel, the nickel content being at least 50% of the alloy, the ratio of the content of the nickel to the sum of the aluminum, the silicon and 2.3 times the titanium being between 13 and 17, and at least a portion of the carbon in the alloy being in the form of graphite.

2. A free machining, age hardenable alloy containing 10% to 45% copper, over 0.25% and up to 5% aluminum, over 0.25% and less than 1% titanium, 0.25% to 5% silicon, 0.2% to 0.35% carbon, 0.05% to 2% manganese, 0.05% to 10% iron, and the balance substantially all nickel, the nickel content being at least 45% of the alloy, the ratio

of the content of the nickel to the sum of the aluminum, the silicon and 2.3 times the titanium being between 11 and 20, and at least a portion of the carbon in the alloy being in the form of graphite.

CLARENCE GEORGE BIEBER.  
MORTIMER FIERCE BUCK.

## REFERENCES CITED

The following references are of record in the file of this patent:

## UNITED STATES PATENTS

|    | Number    | Name    | Date          |
|----|-----------|---------|---------------|
| 15 | 1,572,744 | Mercia  | Feb. 9, 1926  |
|    | 1,610,262 | Cooper  | Dec. 14, 1926 |
|    | 2,048,166 | Pilling | July 21, 1936 |